

# United States Patent [19]

Willis et al.

[11] 3,850,638

[45] Nov. 26, 1974

[54] BENZIMIDAZOLE NUCLEATING AGENTS

[75] Inventors: **Roland George Willis; William Robert Schleigh**, both of Rochester, N.Y.

[73] Assignee: **Eastman Kodak Company**, Rochester, N.Y.

[22] Filed: **Apr. 2, 1973**

[21] Appl. No.: **347,291**

[52] U.S. Cl. .... **96/64, 96/76 R, 96/66 R,**  
96/107;108

[51] Int. Cl. .... **G03c 1/48, G03c 5/24, G03c 5/30,**  
**G03c 1/28**

[58] Field of Search ..... **96/64, 108, 67, 107, 66 R,**  
**96/76 R**

[56]

## References Cited

### UNITED STATES PATENTS

|           |        |                   |        |
|-----------|--------|-------------------|--------|
| 2,497,917 | 2/1950 | Stauffer .....    | 96/64  |
| 3,734,738 | 5/1973 | Kurtz et al. .... | 96/107 |

Primary Examiner—David Klein

Assistant Examiner—Won H. Louie, Jr.

Attorney, Agent, or Firm—C. O. Thomas

[57]

## ABSTRACT

Direct positive photographs are developed in the presence of nucleating amounts of certain benzimidazoles of defined structure. These nucleating agents can be present in the photographic element itself, in the developing solution employed or in a separate bath.

41 Claims, No Drawings

## BENZIMIDAZOLE NUCLEATING AGENTS

## BACKGROUND OF THE INVENTION

## 1. Field of the Invention

The present invention relates to photography and more particularly to novel nucleating agents and direct-positive photographic emulsions.

## 2. Description of the Prior Art

Certain photographic silver halide emulsions are used to produce positive photographic images without a photographic negative.

Generally, these emulsions are termed direct-positive or reversal emulsions and, on exposure, they tend to form latent images predominantly inside the silver halide grains. The production of direct-positive photographic images is secured by selectively fogging the unexposed regions of a direct-positive photographic layer and developing a conventional photographic silver image corresponding to the unexposed, fogged regions. The fogging agent can be included in a "fogging bath" with which the imagewise exposed reversal emulsion is treated prior to image development. Alternatively, the fogging agent can be incorporated directly into the developer solution or it can be included in the reversal emulsion prior to coating a photographic layer.

Ives, in U.S. Pat. Nos. 2,563,785 and 2,588,982 describes the use of hydrazine compounds in direct-positive emulsions of the internal-image type.

Lincoln and Heseltine in U.S. Pat. No. 3,615,615 disclose a variety of aldehyde derivatives of N-acylalkyl heterocyclammonium salts as useful fogging agents in direct-positive, internal-image emulsions.

Belgian patent 774,437 discloses a number of N-substituted heterocyclammonium quaternary salts, including formyl benzothiazolium salts, as nucleating agents for direct-positive, internal-image emulsions.

Stauffer in U.S. Pat. No. 2,497,917 describes developing solutions for direct-positive, internal-image emulsions containing ring compounds. These are heterocyclic nitrogen-containing ring compounds having 5 or 6 atoms in the heterocyclic ring and are so constituted as to increase the maximum density of the positive image obtained in developing solutions capable of producing aerial fog. Typical compounds include benzotriazole, methyl benzotriazole, 5-nitroindazole and 6-nitrobenzimidazole.

British 1,195,838 relates to the use of processing liquids comprising carbazic acid and/or bicarbamic acid and/or at least one water-soluble salt thereof as a fogging compound (or compounds) for partially or wholly replacing an overall exposure step in the production of photographic reversal or direct positive images.

British 1,195,837 relates to a method for the production of direct-positive images by developing in the presence of hydrazine, iodide ions and/or bromide ions.

German 2,015,070 pertains to photographic material for both negative and positive images. The internally ripened grains are fogged.

## SUMMARY OF THE INVENTION

The present invention relates to the use of certain benzimidazoles as nucleating agents in the treatment of internal-image emulsions after exposure, whereby a developable image is produced on the surface of the grains of the emulsion, which image, when developed, has a density inversely proportional to the degree of the initial exposure.

In one aspect, the present invention comprises an improved process for developing direct-positive photographs wherein the improvement comprises carrying out the development in the presence of a nucleating amount of a benzimidazole of the structure:



or the structure:



wherein

R<sub>1</sub>, R<sub>2</sub>, R<sub>4</sub> and R<sub>2</sub>' are independently selected from the group consisting of hydrogen, alkyl, benzyl, phenyl, substituted benzyl, substituted phenyl, acetyl, substituted acetyl, amino and alkylamino;

R<sub>3</sub>, R<sub>4</sub>, R<sub>5</sub>, R<sub>6</sub>, R<sub>3</sub>', R<sub>4</sub>', R<sub>5</sub>' and R<sub>6</sub>' are independently selected from the group consisting of hydrogen, alkyl, alkoxy, nitro, cyano, nitrile amino, amino, benzyl, phenyl, substituted benzyl, substituted phenyl, halogen and ester;

R<sub>7</sub> and R<sub>8</sub> are selected from the group consisting of hydrogen, alkyl, benzyl, phenyl, substituted benzyl, substituted phenyl, amino, alkoxy, cyano, halogen and ester, or are taken together to represent the carbon atoms necessary to complete a 5- or 6-membered cycloalkyl ring; at least one of the groups R<sub>1</sub> and R<sub>7</sub>, R<sub>2</sub> and R<sub>8</sub>, R<sub>1</sub> and R<sub>2</sub>, R<sub>1</sub>' and R<sub>2</sub>' can be taken together to represent the atoms necessary to complete at least one heterocyclic ring.

In a preferred embodiment, at least two of R<sub>1</sub>, R<sub>2</sub>, R<sub>3</sub>, R<sub>4</sub>, R<sub>5</sub> and R<sub>6</sub> are hydrogen.

In one embodiment of this invention, the benzimidazole nucleating agent is present in at least one layer of the photographic element being developed, said layer being in water-permeable association with the silver halide emulsion of the photographic element.

In another embodiment of this invention, the benzimidazole nucleating agent is present in the developer.

Accordingly, the present invention further comprises (1) a photographic element comprising a support having deposited thereon at least one layer comprising a silver halide internal-image photographic emulsion and at least one layer in water-permeable association with said silver halide layer comprising a nucleating amount of a benzimidazole and (2) a photographic developer composition containing a nucleating amount of a benzimidazole; said benzimidazole being of the structure:



or the structure:



wherein

R<sub>1</sub>, R<sub>2</sub>, R<sub>1</sub>' and R<sub>2</sub>' are independently selected from the group consisting of hydrogen, alkyl, benzyl, phenyl, substituted benzyl, substituted phenyl, acetyl, substituted acetyl, amino and alkylamino; R<sub>3</sub>, R<sub>4</sub>, R<sub>5</sub>, R<sub>6</sub>, R<sub>3</sub>', R<sub>4</sub>', R<sub>5</sub>' and R<sub>6</sub>' are independently selected from the group consisting of hydrogen, alkyl, alkoxy, nitro, cyano, nitrile amino, amino, substituted amino, benzyl, phenyl, substituted benzyl, substituted phenyl, halogen and ester, R<sub>7</sub> and R<sub>8</sub> are selected from the group consisting of hydrogen, alkyl, benzyl, phenyl, substituted benzyl, substituted phenyl, amino, alkoxy, cyano, halogen and ester, or are taken together to represent the carbon atoms necessary to complete a 5- or 6-membered cycloalkyl ring; at least one of the groups R<sub>1</sub> and R<sub>7</sub>, R<sub>2</sub> and R<sub>8</sub>, R<sub>1</sub> and R<sub>2</sub>, R<sub>1</sub>' and R<sub>2</sub>' can be taken together to represent the atoms necessary to complete at least one heterocyclic ring. In preferred embodiments, at least two of R<sub>1</sub>, R<sub>2</sub>, R<sub>3</sub>, R<sub>4</sub>, R<sub>5</sub> and R<sub>6</sub> are hydrogen.

#### DESCRIPTION OF THE PREFERRED EMBODIMENTS

As stated above, the benzimidazole nucleating agents employed in the practice of this invention are of the structure:



or the structure:



In these structural formulae, R<sub>1</sub>, R<sub>2</sub>, R<sub>1</sub>' and R<sub>2</sub>' can be the same or different and can be hydrogen; alkyl, for

example an alkyl group having from 1 to 12 carbon atoms and, preferably,

a lower alkyl group such as one having from 1 to 4 carbon atoms, e.g. methyl, ethyl, propyl, isopropyl, butyl, isobutyl, sec.-butyl and tert.-butyl; benzyl, substituted benzyl, e.g., halogen, substituted benzyl, alkyl, especially lower alkyl, substituted benzyl and the like; phenyl; substituted phenyl, e.g. halogen substituted phenyl, alkyl, especially lower alkyl, substituted phenyl, alkoxy,

especially lower alkoxy, substituted phenyl and the like; acetyl; substituted acetyl, e.g. halogen substituted acetyl, phenyl substituted acetyl, substituted phenyl substituted acetyl, and the like; amino, including primary, secondary and tertiary amino, particularly alkyl-

15 amino, which term is intended to include both monoalkylamino and dialkylamino, wherein the alkyl group or groups can have from 1 to 12 carbon atoms, but preferably are lower alkyl groups of from 1 to 4 carbon atoms.

20 R<sub>3</sub>, R<sub>4</sub>, R<sub>5</sub>, R<sub>6</sub>, R<sub>3</sub>', R<sub>4</sub>', R<sub>5</sub>' and R<sub>6</sub>' can be the same or different and can be hydrogen; alkyl, as described above for R<sub>1</sub>, etc.; alkoxy, for example, an alkoxy group having from 1 to 12 carbon atoms and, preferably a lower alkoxy group such as one having from 1 to 4 carbon atoms, e.g., methoxy, ethoxy, propoxy, isopropoxy, butoxy, isobutoxy, sec.-butoxy and tert.-butoxy; nitro;

25 cyano; nitrile amino, i.e. N ≡ C-NH—; amino, including primary, secondary and tertiary amino; substituted amino, including monoalkyl, dialkyl, monoaryl and diaryl substituted amino wherein alkyl can be as described for R<sub>1</sub>, etc. and aryl, which term is intended to include substituted aryl, is phenyl, tolyl, xylyl, chlorophenyl, bromophenyl and the like; benzyl, phenyl, substituted benzyl and substituted phenyl as described above for R<sub>1</sub>, etc.; halogen, i.e., chloro, fluoro, bromo or iodo; and ester, i.e.,

30 35

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040</

5



Spiro[5-nitrobenzimidazoline-2,1'-cyclohexane]



Spiro[5-methoxybenzimidazoline-2,1'-cyclohexane]



Spiro[benzimidazoline-2,1'-(4'-methylcyclohexane)]



1,3-Bistrifluoroacetyl-2,3-dihydrobenzimidazole



5-Methoxy-1,3-bistrifluoroacetyl-2,3-dihydrobenzimidazole



5,6-Dimethyl-1,3-bistrifluoroacetyl-2,3-dihydrobenzimidazole

6



10 4-Benzyl-2,3,3a,4-tetrahydro-1H-pyrrolo-[1,2-a]benzimidazole



20 Benzimidazoline-2-spiro-1'-cyclohexane-4'-spiro-2''-benzimidazoline



1,3-Dimethyl-2-phenyl-1,2-dihydrobenzimidazole



45 1,3-Dimethyl-2-(4'-methoxyphenyl)-1,2-dihydrobenzimidazole



55 1,3,5-Trimethyl-2-phenyl-1,2-dihydrobenzimidazole



65 1,3,5,6-Tetramethyl-2-phenyl-1,2-dihydrobenzimidazole



5-Chloro-1,3-dimethyl-2-phenyl-1,2-dihydrobenzimidazole



1,3,5-Trimethyl-2-(4'-methoxyphenyl)-1,2-dihydrobenzimidazole



1,3,5,6-Tetramethyl-2-(4'-methoxyphenyl)-1,2-dihydrobenzimidazole



5-Chloro-1,3-dimethyl-2-(4'-methoxyphenyl)-1,2-dihydrobenzimidazole



1,3-Dimethyl-2-(4'-chlorophenyl)-1,2-dihydrobenzimidazole

The above-described benzimidazoles are extremely advantageous as incorporated nucleating agents or fogging agents in silver halide reversal or direct-positive

emulsions utilized in photographic elements designed for reversal processing to prepare direct-positive photographic images without an intermediate developed negative image. Typical of such direct-positive emulsions are those that form latent images predominantly inside the silver halide grains.

The photographic emulsions generally used in reversal processes are gelatino-silver halide emulsions such as silver bromide, silver bromoiodide, silver chloride, silver chloroiodide, silver chlorobromooiodide or silver chlorobromide emulsions. They need not contain sensitizing dyes although certain of such dyes can be added to reversal emulsions to widen spectral sensitization. Advantageous sensitizing dyes would include those described in U.S. Pat. No. 2,497,876, especially between column 2, line 15 and column 4, line 20. Internal latent image-forming emulsions are typically undigested or if digested, the digestion is carried out without the use of surface chemical sensitizers. An emulsion of this type, known as Burton's emulsion, is described in Wall "Photographic Emulsions," 1927, pp. 52 and 53. Other types of suitable reversal emulsions are the internal latent image emulsions described in Davey and Knott, U.S. Pat. No. 2,592,250 or those described in Belgian Patent 780,538, issued Mar. 31, 1972.

An internal latent image-forming emulsion can be prepared by first forming in one or more stages silver salt grains consisting at least partly of a silver salt which is more soluble in water than silver bromide, subsequently converting at least part of the grains to silver bromide or silver bromoiodide, ripening, preferably in the absence of ammonia, and then either washing out some of the soluble salts or washing out the whole of the soluble salts, followed by the addition of soluble salts such as soluble chloride, bromide or iodide to prepare a composite silver chlorobromide, bromoiodide or chlorobromooiodide reversal emulsion. Suitable silver chlorobromide internal image emulsions also can be prepared by simultaneously adding an aqueous solution of silver nitrate and an aqueous solution containing potassium chloride and potassium bromide to an agitated aqueous gelatin solution as described in Example 4 of Luckey et al., U.S. Pat. No. 2,996,382.

An "internal latent image" type of silver halide emulsion can be defined as one which, when a test portion is exposed to a light intensity scale for a fixed time up to about 1 second and developed for 4 minutes at 20°C in an ordinary "surface" developer (one which develops an image only on the surface of the grains of an "internal latent image emulsion" which developer type is exemplified by one having the formula:

|                             |           |
|-----------------------------|-----------|
| p-hydroxyphenylglycine      | 10 grams  |
| sodium carbonate (crystals) | 100 grams |
| water to                    | 1 liter)  |

exhibits a maximum density not greater than 1/5 the maximum density obtained when the same emulsion is equally exposed and developed for 3 minutes at 20°C in an "internal" type developer (one which develops an image inside the grains of an "internal latent image emulsion," which developer type is exemplified by one having the formula:

|                                  |           |
|----------------------------------|-----------|
| hydroquinone                     | 15 grams  |
| monomethyl-p-aminophenol sulfate | 15 grams  |
| sodium sulfite (anhydrous)       | 50 grams  |
| potassium bromide                | 10 grams  |
| sodium hydroxide                 | 25 grams  |
| sodium thiosulfate (crystals)    | 20 grams  |
| water to                         | 1 liter). |

Preferably the maximum density obtained with the "surface" developer is not greater than 1/10 the maximum density obtained when the same emulsion is developed in the "internal" type developer. Stated conversely, an "internal latent image" emulsion, when developed in an "internal type developer" exhibits a maximum density at least 5 and preferably at least 10 times the maximum density obtained when the emulsion is exposed in the same way and developed in a "surface" developer.

The subject benzimidazoles that operate advantageously as nucleating agents or fogging agents in internal latent image-forming (reversal) emulsions are conveniently added to a silver halide reversal emulsion, such as, for example, those described in U.S. Pat. Nos. 2,566,180 or 2,592,250 in amounts designed to produce adequate fog in the form of minute surface development sites which foster the production of direct-positive images upon development.

Generally, the fogging agents can be incorporated in at least one layer of the photographic element in water-permeable association with the silver halide emulsion or they can be contacted with the emulsion before or during development such as by a pre-bath or incorporating the fogging agent in the developer composition; however, the fogging agents are preferably located in at least one layer of the element and in a highly preferred embodiment they are located in the silver halide emulsion layer. Concentrations of from about 75 to about 1,500 mg. of the subject fogging agents per mole of silver in the silver halide emulsion are useful, with from about 90 to about 1,200 mg. of said compounds or agents per mole of silver being preferred. It is most preferred to employ from about 90 to about 150 mg. of nucleating agent per mole of silver. These ratios are according to conventional practice, however, and with either particular reversal emulsions, fogging compounds of varying chemical activity, or varying processing conditions, more widely varying fogging agent concentrations can be advantageously used.

The silver halide emulsions employed in the practice of this invention are developed in a silver halide surface developer in the presence of the fogging agents of this invention to provide good positive images. The fogging agents can be incorporated in at least one layer of the silver halide element, which layer is in water-permeable association with the silver halide emulsion, or they can be contacted with said silver halide emulsion by a separate bath or simultaneously with the surface developer composition by incorporating them into the developer composition. Generally, the fogging agents of this invention provide nucleation or fog specks which initiate development of the silver halide in the unexposed areas before initiating substantial development in the exposed areas of an internal-image emulsion in a surface developer.

Silver halide emulsions into which the benzimidazole nucleating agents of this invention are advantageously incorporated typically contain other chemical addenda such as, for example, carrier vehicles, spectral sensitizing dyes, coating aids, brighteners, hardeners, developing agents and the like. Desirable carrier vehicles include any of the hydrophilic, water-permeable binding materials suitable for this purpose. Suitable materials include gelatin, colloidal albumin, polyvinyl compounds, cellulose derivatives, acrylamide polymers and the like, alone or in combination and admixture. The

binding agents for the emulsion layer of the photographic element can also contain dispersed polymerized vinyl compounds. Certain of such compounds are disclosed, for example, in U.S. Pat. Nos. 3,142,468 of Nottorf issued July 28, 1964; 3,193,386 of White issued July 6, 1965; 3,062,672 of Houck et al. issued Nov. 6, 1962; and 3,220,844 of Houck et al. issued Nov. 30, 1965; and include the water-insoluble polymers and latex copolymers of alkyl acrylates and methacrylates, acrylic acid sulfoalkyl acrylates or methacrylates and the like.

Spectral sensitizing dyes useful in sensitizing the silver halide emulsions employed in this invention are described in, for example, U.S. Pat. No. 2,562,632 of Brooker and White issued Oct. 24, 1950 and U.S. Pat. No. 2,503,776 of Sprague issued Apr. 11, 1950. Spectral sensitizers which can be used are the cyanines, merocyanines, complex (trinuclear) cyanines, complex (trinuclear) merocyanines, styryls and hemicyanines.

The photographic silver halide emulsions or coatings employed herein can also contain non-ionic, anionic and/or amphoteric coating aids. Some useful coating aids include, for example, saponin, alkyl substituted aryloxyalkylene ethyl sulfonates of the type described in U.S. Pat. No. 2,600,831 issued June 17, 1952, maleopimаратes of the type described in U.S. Pat. No. 2,823,123, issued Feb. 11, 1958, taurine derivatives of the type described in U.S. Pat. No. 2,739,891 issued on Mar. 27, 1956, and alkyl aminopropionates of the type described in U.S. Pat. No. 3,133,816 issued May 19, 1964. Typical of still other good coating aids and surfactants which can be employed in the emulsions of this invention include the alkylphenoxy poly(hydroxyalkylene oxides) such as alkylphenoxy poly(glycidols) having from about 5 to about 12 glycidol units, for example, such as those disclosed in British Patent 1,022,878 issued Mar. 16, 1966.

Advantageous brighteners typically include compounds containing at least one heterocyclic five or six membered ring such as derivatives of stilbene, stilbene-triazole, triazine stilbene, coumarin, triazinylamino coumarin, oxazole, benzidene, benzimidazole, benzothiazole, benzoxazole, pyrazoline, naphthalic acid imide, etc. Exemplary brighteners include such compounds as those described in U.S. Pat. No. 2,933,390 and U.S. Pat. No. 3,406,070.

As well as including the above-mentioned addenda, the silver halide emulsions employed in this invention can be hardened with any suitable hardener or combination such as, e.g., formaldehyde, mucochloric acid, glutaraldehyde, maleic dialdehyde, aldehyde hardeners, aziridine hardeners, hardeners which are derivatives of dioxane, vinyl sulfones, oxypolysaccharides such as oxystarch, oxy plant gums, inorganic hardeners such as chromium salts, and the like. Developing agents of the types suitable for inclusion in a silver halide emulsion are described hereinbelow.

To prepare direct-positive photographic elements that can be reversal processed, an internal latent image-forming silver halide emulsion such as described hereinabove, is coated onto a typical photographic support material and dried. Advantageous support materials include conventional photographic film base materials like cellulose esters such as cellulose acetate, cellulose triacetate, cellulose acetate butyrate, etc., polyolefins like polyethylene and polypropylene, polycarbonates, polyesters such as poly(ethylene terephthal-

ate) as well as metals such as zinc and aluminum and paper including polyethylene and polypropylene coated papers. Other support materials that are suitably used herein are known in the art.

The nucleating agents of the invention can be used in reversal color as well as black-and-white silver halide emulsions. The preparation of color reversal photographic elements is conveniently accomplished by employing cyan, magenta and yellow color-forming couplers contiguous to silver halide emulsions capable of recording light substantially complementary in color to the color of dye produced with the respective couplers on color development as described in U.S. Pat. No. 3,227,550 and 3,227,552. Spectral sensitizing dyes can be used to sensitize the silver halide in the usual manner. In a multilayer element, the red-recording emulsion layer can contain a coupler such as 5-(*p*-amylphenoxy benzene sulfonamino)-1-naphthol, the green-recording emulsion layer, a coupler like 2-cyanoacetyl-5-(*p*-sec. amylbenzoylamino) coumarone and the blue-recording emulsion layer, a coupler such as N-amyl-*p*-benzoylacetamino benzene sulfonate. Additional couplers are well known in the art. If desired, the color couplers can be incorporated into the developer solution, as described in Mannes et al., U.S. Pat. No. 2,252,718 and Glass et al., U.S. Pat. No. 2,507,154, such an arrangement necessitating multiple exposures and color developing steps.

After an imagewise exposure, the direct-positive photographic elements containing the subject nucleating agents are immersed in a conventional surface developer solution having relatively low solvent action on silver halide whereupon a positive photographic image is formed. Such surface developers can advantageously contain image-enhancing compounds which increase maximum image density and lower minimum image density such as the benzotriazoles described in Stauffer, U.S. Pat. No. 2,497,917.

If color images are to be prepared, the developer solution typically contains a *o*-phenylenediamine color developing agent such as a 4-amino-N-dialkylaniline like those described in Mees, "The Theory of the Photographic Process," 3rd Ed. (1966) pp. 294-295. With a color developer, one or more colored dye images are produced depending upon the construction of the particular photographic element. In polychromatic color elements, cyan, magenta and yellow dye images are typically produced in the red sensitive, green sensitive and blue sensitive layers, respectively. Remaining silver is first converted to a soluble silver salt and removed in the usual way by treatment with a fixing agent such as sodium thiosulfate.

The following examples are included for a further understanding of the invention:

#### EXAMPLE 1

##### *Spiro[benzimidazoline-2,1'-cyclohexane]*

This compound is prepared according to the procedure of R. Garner, G. V. Garner, and H. Suschitzky, *J. Chem. Soc. (C)*, 825 (1970).

A mixture of *o*-phenylenediamine (10.80 g, 0.1 mole) and cyclohexanone (9.82 g, 0.1 mole) in tetrahydrothiophene-1,1-dioxide (30 ml) is heated 90 minutes on a steam bath. The hot mixture is poured into water. The solid that separates is collected, washed first with water, then with a small volume of ethyl alcohol, and finally with ligroin (b.p. 35°-55°C). The

washed material is air-dried to yield a yellow solid, 10.52 g, m.p. 135°C (dec.). Recrystallization from ethyl alcohol gives 5.10 g of yellow needles (27 percent yield) which decompose at 144°C.

#### EXAMPLE 2

##### *Spiro[5-nitrobenzimidazoline-2,1'-cyclohexane]*

Example 1 is repeated except that 4-nitro-*o*-phenylenediamine is substituted on an equimolar basis for the *o*-phenylenediamine employed therein. A product having a melting point in the range 160°-164°C is obtained in 57 percent yield.

#### EXAMPLE 3

##### *Spiro[5-methoxybenzimidazoline-2,1'-cyclohexane]*

Example 1 is repeated except that 4-methoxy-*o*-phenylenediamine is substituted on an equimolar basis for the *o*-phenylenediamine employed therein. A product having a melting point in the range 104°-106°C is obtained in 28 percent yield.

#### EXAMPLE 4

##### *Spiro[benzimidazoline-2,1'-(4-methylcyclohexane)]*

Example 1 is repeated except that 4-methylcyclohexanone is substituted on an equimolar basis for the cyclohexanone employed therein. A product having a melting point in the range 108°-111°C is obtained in 60 percent yield.

#### EXAMPLE 5

##### 1,3-Bistrifluoroacetyl-2,3-dihydrobenzimidazole

A suspension of PtO<sub>2</sub> (1.0 g) in trifluoroacetic anhydride (100 g) is shaken under hydrogen for 5 minutes, then cooled. The reaction vessel is flushed with nitrogen, then benzimidazole (2.36 g, 0.02 mole) is added while the vessel is cooled in an ice bath. The resulting solution is shaken under hydrogen until uptake is complete, then it is filtered and the filtrate concentrated. The residue is recrystallized from ethyl alcohol providing colorless crystals having a melting point of 130°-132°C in 66 percent yield.

#### EXAMPLE 6

##### 5-Methoxy-1,3-bistrifluoroacetyl-2,3-dihydrobenzimidazole

Example 5 is repeated except that 5-methoxybenzimidazole is substituted on an equimolar basis for the benzimidazole employed therein. A product having a melting point in the range 104°-106°C is obtained in 33 percent yield.

#### EXAMPLE 7

##### 5,6-Dimethyl-1,3-bistrifluoroacetyl-2,3-dihydrobenzimidazole

Example 5 is repeated except that 5,6-dimethylbenzimidazole is substituted on an equimolar basis for the benzimidazole employed therein. A product having a melting point in the range 118°-121°C is obtained in 57 percent yield.

#### EXAMPLE 8

A 16 mm by 12 inch sample of a photographic element containing an internal-image silver halide emulsion of the type described in Belgian Patent 780,538 issued Mar. 31, 1972 was exposed (0-6 step tablet, 3,000°K, 750W) for 1 second and immersed in a 1-liter bath containing 100 mg of the compound of Example

1 at a pH of 12.9 at 68°F (20°C) for 1 minute, washed in a 3 percent aqueous acetic acid solution for 2 minutes, in distilled water for 5 minutes and developed in the following surface developer for 5 minutes:

|                                                        |        |
|--------------------------------------------------------|--------|
| L-ascorbic acid<br>(N-methyl-p-aminophenol<br>sulfate) | 10 g.  |
| Sodium metaborate . 4H <sub>2</sub> O                  | 2.5 g. |
| KBr                                                    | 35 g.  |
| Water to make 1 liter<br>pH 9.8 at 75°F                | 1 g.   |

All solutions were deaerated before use and nitrogen burst agitation was employed throughout the process. The strip was bathed for one minute in 3 percent acetic

ample 1. The treated sample was bathed in 3 percent acetic acid for one minute, fixed in Kodak Fixing Bath F-5 for 10 minutes, water washed for 10 minutes and dried. The photographic results obtained are shown in Table I.

#### EXAMPLES 10-15

The procedure of Example 9 was repeated with each of the compounds of Examples 2 through 7. The results obtained are also shown in Table I. In each instance, a positive image was obtained, and the discrimination is reflected by a comparison of the silver formed in the unexposed and exposed areas of the test samples.

TABLE I

| Compound of<br>Example No. | Structure<br>R'<br>R''          | Silver formed (mg/ft <sup>2</sup> ) |                            |
|----------------------------|---------------------------------|-------------------------------------|----------------------------|
|                            |                                 | Exposed<br>(Log E=1.70)             | Unexposed<br>(Log E=-0.70) |
| General formula            |                                 |                                     |                            |
| 1                          | H H                             | 1                                   | 23                         |
| 2                          | NO <sub>2</sub> H               | 7                                   | 13*                        |
| 3                          | CH <sub>3</sub> O H             | 5                                   | 23                         |
| 4                          | H CH <sub>3</sub>               | 7                                   | 25                         |
| General formula            |                                 |                                     |                            |
| 5                          | H H                             | 2                                   | 18*                        |
| 6                          | CH <sub>3</sub> O H             | 12                                  | 27                         |
| 7                          | CH <sub>3</sub> CH <sub>3</sub> | 5                                   | 24*                        |

\*Development time of 3 min., all others 1 min.

acid and 10 minutes in Kodak Fixing Bath F-5 (see 55 Handbook of Chemistry and Physics, Forty-First Edition, pp. 3,315-3,316), then washed with water for 10 minutes and dried giving a positive image of developed silver. Omission of the pretreatment with the solution containing the compound of Example 1 gave no image. 60

#### EXAMPLE 9

An exposed sample of the photographic element identified in Example 8 was treated with a surface developer comprising 4-amino-N-ethyl-N-β-hydroxyethylaniline (2.78 g. in 1 liter of 0.1 N potassium hydroxide) and 100 mg. of the compound of Ex- 65

#### EXAMPLE 16

4-Benzyl-2,3,3a,4-tetrahydro-1H-pyrrolo-[1,2-a]benzimidazole



A solution of 7.69 gms. of N-(o-nitrophenyl) pyrrolidine in 75 ml. of ethanol containing 1 gm. of 10 percent palladium on charcoal was shaken under hydrogen until the uptake ceased. The solution was filtered and the filtrate was treated first with 0.04 mole of benzaldehyde and then with a few drops of concentrated HCl. The mixture was stirred overnight under a nitrogen atmosphere and then was concentrated. The residue was distilled in vacuo to yield 5.34 grams of a pale yellow oil having a boiling point of 153°C at 0.1 mm Hg. The boiling point of this compound was reported by Grantham et al. in J. Chem. Soc. (C), 1438 (1969) to be 164°C at 0.6 mm Hg.

## EXAMPLE 17

Benzimidazoline-2-spiro-1'-cyclohexane-4'-spiro-2''-benzimidazoline



This compound was prepared according to the procedure of Example 1 using 0.1 mole of o-phenylenediamine and 0.05 mole of cyclohexane-1,4-dione. Water was the solvent employed. The product was obtained in 90 percent yield and had a melting point of 230°-233°C (dec.).

## EXAMPLE 18

1,3-Dimethyl-2-(4'-methoxyphenyl)-1,2-dihydrobenzimidazole



A mixture of 5.12 gms. of N,N'-dimethyl-o-phenylenediamine and 5.12 gms. of anisaldehyde in 20 ml. of ethanol was allowed to stand for three days at room temperature under a nitrogen atmosphere. The resulting crystalline material was collected and recrystallized from ethanol to give 4.15 gms. of colorless crystals, a 43 percent yield. The melting point of the crystals was 107°-109°C.

## EXAMPLES 19-21

Samples of the exposed photographic element identified in Example 8 were treated according to the procedure of Example 8 except that the nucleating agents were the compounds of Examples 16, 17 and 18, respectively. In each case, well-defined positive images similar to those of Examples 8-15 were obtained.

The invention has been described in detail with particular reference to certain preferred embodiments thereof, but it will be understood that variations and modifications can be effected within the spirit and scope of the invention.

We claim:

1. In a process for developing internal latent image silver halide emulsions to produce direct positive photo-

tographs, the improvement which comprises carrying out the development with a surface silver halide developer in contact with a nucleating amount of a benzimidazole of the structure:



or the structure:



wherein

R<sub>1</sub>, R<sub>2</sub>, R'<sub>1</sub> and R'<sub>2</sub> are independently selected from the group consisting of hydrogen, alkyl, benzyl, phenyl, halogen or alkyl substituted benzyl, halogen, alkoxy or alkyl substituted phenyl, acetyl, halogen or phenyl substituted acetyl, and amino;

R<sub>3</sub>, R<sub>4</sub>, R<sub>5</sub>, R<sub>6</sub>, R'<sub>3</sub>, R'<sub>4</sub>, R'<sub>5</sub> and R'<sub>6</sub>' are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the group R<sub>1</sub> and R<sub>7</sub>, R<sub>2</sub> and R<sub>8</sub>, R<sub>1</sub> and R<sub>2</sub>, R'<sub>1</sub> and R'<sub>2</sub> can be taken together to represent the atoms necessary to complete at least one heterocyclic ring.

2. The process of claim 1 wherein the benzimidazole nucleating agent is present in at least one layer of the photographic element being developed.

3. The process of claim 1 wherein the benzimidazole nucleating agent is present in the developer employed to develop the direct positive photographs.

4. The process of claim 1 wherein at least two of R<sub>1</sub>, R<sub>2</sub>, R<sub>3</sub>, R<sub>4</sub>, R<sub>5</sub> and R<sub>6</sub> are hydrogen.

5. In a process for developing internal latent image silver halide emulsions to produce direct positive photographs, the improvement which comprises carrying out the development with a surface silver halide developer in the presence of from about 75 to about 1,500 mg. per mole of silver in the silver halide emulsion of a benzimidazole of the structure:



wherein

R<sub>1</sub> and R<sub>2</sub> are independently selected from the group consisting of hydrogen, alkyl, benzyl, phenyl, halogen or alkyl substituted benzyl, halogen, alkoxy or alkyl substituted phenyl, acetyl, halogen or phenyl substituted acetyl, and amino;

R<sub>3</sub>, R<sub>4</sub>, R<sub>5</sub> and R<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the groups R<sub>1</sub> and R<sub>7</sub>, R<sub>2</sub> and R<sub>8</sub>, R<sub>1</sub> and R<sub>2</sub> can be taken together to represent the atoms necessary to complete at least one heterocyclic ring.

6. In a process for developing internal latent image silver halide emulsions to produce direct positive photographs, the improvement which comprises carrying out the development with a surface silver halide developer in the presence of a nucleating amount of a benzimidazole of the structure:



wherein

R<sub>1</sub>, R<sub>2</sub>, R<sub>1'</sub> and R<sub>2'</sub> are independently selected from the group consisting of hydrogen, alkyl, benzyl, phenyl, halogen or alkyl substituted benzyl, halogen, alkyl or alkoxy substituted phenyl, acetyl, halogen or phenyl substituted acetyl, and amino;

R<sub>3</sub>, R<sub>4</sub>, R<sub>5</sub>, R<sub>6</sub>, R<sub>3'</sub>, R<sub>4'</sub>, R<sub>5'</sub> and R<sub>6'</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

at least one of the groups R<sub>1</sub> and R<sub>2</sub>, R<sub>1'</sub> and R<sub>2'</sub> can be taken together to represent the atoms necessary to complete at least one heterocyclic ring.

7. The process of claim 5 wherein the benzimidazole is of the structure:



wherein R<sub>4</sub> is hydrogen, nitro or alkoxy and R<sub>11</sub> is hydrogen or lower alkyl.

8. The process of claim 7 wherein the benzimidazole is spiro [benzimidazoline-2,1'-cyclohexane].

9. The process of claim 7 wherein the benzimidazole is spiro [5-nitrobenzimidazoline 2,1'-cyclohexane].

10. The process of claim 7 wherein the benzimidazole is spiro [5-methoxybenzimidazoline-2,1'-cyclohexane].

11. The process of claim 7 wherein the benzimidazole is spiro [benzimidazoline-2,1'-(4'-methylcyclohexane)].

12. The process of claim 5 wherein the benzimidazole is of the structure:



wherein R<sub>1</sub> and R<sub>2</sub> are halogen or phenyl substituted acetyl and R<sub>4</sub> and R<sub>5</sub> are independently selected from the group consisting of hydrogen, alkyl and alkoxy.

13. The process of claim 12 wherein the benzimidazole is 1,3-bistrifluoroacetyl-2,3-dihydrobenzimidazole.

14. The process of claim 12 wherein the benzimidazole is 5-methoxy-1,3-bistrifluoroacetyl-2,3-dihydrobenzimidazole.

15. The process of claim 12 wherein the benzimidazole is 5,6-dimethyl-1,3-bistrifluoroacetyl-2,3-dihydrobenzimidazole.

30 16. A photographic element comprising a support having deposited thereon at least one layer comprising a silver halide internal-image photographic emulsion and at least one layer in water-permeable association with said silver halide layer comprising a nucleating 35 amount of benzimidazole of the structure:



45 or the structure:



55 wherein

R<sub>1</sub>, R<sub>2</sub>, R<sub>1'</sub> and R<sub>2'</sub> are independently selected from the group consisting of hydrogen, alkyl, benzyl, phenyl, halogen or alkyl substituted benzyl, halogen, alkoxy or alkyl substituted phenyl, acetyl, halogen or phenyl substituted acetyl, and amino;

R<sub>3</sub>, R<sub>4</sub>, R<sub>5</sub>, R<sub>6</sub>, R<sub>3'</sub>, R<sub>4'</sub>, R<sub>5'</sub> and R<sub>6'</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the groups R<sub>1</sub> and R<sub>7</sub>, R<sub>2</sub> and R<sub>8</sub>, R<sub>1</sub> and R<sub>2</sub>, R'<sub>1</sub> and R'<sub>2</sub> can be taken together to represent the atoms necessary to complete at least one heterocyclic ring.

17. The element of claim 16 wherein at least two of R<sub>1</sub>, R<sub>2</sub>, R<sub>3</sub>, R<sub>4</sub>, R<sub>5</sub> and R<sub>6</sub> are hydrogen.

18. A photographic element comprising a support having deposited thereon at least one layer comprising a silver halide internal-image photographic emulsion and at least one layer in water-permeable association with said silver halide layer comprising from about 75 to about 1,500 mg per mole of silver in the silver halide emulsion of a benzimidazole of the structure:



wherein

R<sub>1</sub> and R<sub>2</sub> are independently selected from the group consisting of hydrogen, alkyl, benzyl, phenyl, halogen or alkyl substituted benzyl, halogen, alkyl or alkoxy substituted phenyl, acetyl, halogen or phenyl substituted acetyl, and amino;

R<sub>3</sub>, R<sub>4</sub>, R<sub>5</sub> and R<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the groups R<sub>1</sub> and R<sub>7</sub>, R<sub>2</sub> and R<sub>8</sub>, R<sub>1</sub> and R<sub>2</sub>, R'<sub>1</sub> and R'<sub>2</sub> can be taken together to represent the atoms necessary to complete at least one heterocyclic ring.

19. A photographic element comprising a support having deposited thereon at least one layer comprising a silver halide internal-image photographic emulsion and at least one layer in water-permeable association with said silver halide layer comprising a nucleating amount of a benzimidazole of the structure:



wherein

R<sub>1</sub>, R<sub>2</sub>, R'<sub>1</sub> and R'<sub>2</sub> are independently selected from the group consisting of hydrogen, alkyl, benzyl,

phenyl, halogen or alkyl substituted benzyl, halogen, alkyl or alkoxy substituted substituted phenyl, acetyl, halogen or phenyl substituted acetyl, and amino;

5 R<sub>3</sub>, R<sub>4</sub>, R<sub>5</sub>, R<sub>6</sub>, R'<sub>3</sub>, R'<sub>4</sub>, R'<sub>5</sub> and R'<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

at least one of the groups R<sub>1</sub> and R<sub>2</sub>, R'<sub>1</sub> and R'<sub>2</sub> can be taken together to represent the atoms necessary to complete at least one heterocyclic ring.

20. The element of claim 18 wherein the benzimidazole is of the structure:



wherein R<sub>4</sub> is hydrogen, nitro or alkoxy and R<sub>11</sub> is hydrogen or lower alkyl.

25 21. The element of claim 20 wherein the benzimidazole is spiro [benzimidazoline-2,1'-cyclohexane].

22. The element of claim 20 wherein the benzimidazole is spiro [5-nitrobenzimidazoline-2,1'-cyclohexane].

30 23. The element of claim 20 wherein the benzimidazole is spiro [5-methoxybenzimidazoline-2,1'-cyclohexane].

24. The element of claim 20 wherein the benzimidazole is spiro [benzimidazoline-2,1'-(4'-methylcyclohexane)].

35 25. The element of claim 18 wherein the benzimidazole is of the structure:



wherein R<sub>1</sub> and R<sub>2</sub> are halogen or phenyl substituted acetyl and R<sub>4</sub> and R<sub>5</sub> are independently selected from the group consisting of hydrogen, alkyl and alkoxy.

50 26. The element of claim 25 wherein the benzimidazole is 1,3-bistrifluoroacetyl-2,3-dihydrobenzimidazole.

27. The element of claim 25 wherein the benzimidazole is 5-methoxy-1,3-bistrifluoroacetyl-2,3-dihydrobenzimidazole.

55 28. The element of claim 25 wherein the benzimidazole is 5,6-dimethyl-1,3-bistrifluoroacetyl-2,3-dihydrobenzimidazole.

29. A photographic silver halide surface developer 60 composition containing a nucleating amount of a benzimidazole of the structure:



or the structure:



wherein

R<sub>1</sub>, R<sub>2</sub>, R'<sub>1</sub> and R'<sub>2</sub> are independently selected from the group consisting of hydrogen, alkyl, benzyl, phenyl, halogen or alkyl substituted benzyl, halogen, alkyl or alkoxy substituted phenyl, acetyl, halogen or alkyl substituted acetyl, and amino;

R<sub>3</sub>, R<sub>4</sub>, R<sub>5</sub>, R<sub>6</sub>, R'<sub>3</sub>, R'<sub>4</sub>, R'<sub>5</sub> and R'<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the groups R<sub>1</sub> and R<sub>7</sub>, R<sub>2</sub> and R<sub>8</sub>, R<sub>1</sub> and R<sub>2</sub>, R'<sub>1</sub> and R'<sub>2</sub> can be taken together to represent the atoms necessary to complete at least one heterocyclic ring.

30. The developer of claim 29 wherein at least two of R<sub>1</sub>, R<sub>2</sub>, R<sub>3</sub>, R<sub>4</sub>, R<sub>5</sub> and R<sub>6</sub> are hydrogen.

31. A photographic silver halide surface developer composition containing from about 75 to about 1,500 mg per mole of silver in the silver halide emulsion to be developed of benzimidazole of the structure:



R<sub>1</sub> and R<sub>2</sub> are independently selected from the group consisting of hydrogen, alkyl, benzyl, phenyl, phenyl or halogen substituted benzyl, halogen, alkyl or alkoxy substituted phenyl, acetyl, halogen or alkyl substituted acetyl, and amino;

R<sub>3</sub>, R<sub>4</sub>, R<sub>5</sub> and R<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

R<sub>7</sub> and R<sub>8</sub> are selected from the group consisting of hydrogen, alkyl, benzyl, phenyl, halogen or alkyl substituted benzyl, halogen, alkyl or alkoxy substituted phenyl, amino, alkoxy, cyano, halogen and ester, or are taken together to represent the carbon atoms necessary to complete a 5- or 6-membered cycloalkyl ring;

at least one of the groups R<sub>1</sub> and R<sub>7</sub>, R<sub>2</sub> and R<sub>8</sub>, R<sub>1</sub> and R<sub>2</sub> can be taken together to represent the atoms necessary to complete at least one heterocyclic ring.

32. A photographic silver halide surface developer composition containing a nucleating amount of a benzimidazole of the structure:



wherein

R<sub>1</sub>, R<sub>2</sub>, R'<sub>1</sub> and R'<sub>2</sub> are independently selected from the group consisting of hydrogen, alkyl, benzyl, phenyl, halogen or alkyl substituted benzyl, substituted phenyl, acetyl, halogen or phenyl substituted acetyl, and amino;

R<sub>3</sub>, R<sub>4</sub>, R<sub>5</sub>, R<sub>6</sub>, R'<sub>3</sub>, R'<sub>4</sub>, R'<sub>5</sub> and R'<sub>6</sub> are independently selected from the group consisting of hydrogen, alkyl, alkoxy, nitro, cyano, nitrile amino, amino, benzyl, phenyl, halogen or alkyl substituted benzyl, halogen, alkyl or alkoxy substituted phenyl, halogen and ester;

at least one of the groups R<sub>1</sub> and R<sub>2</sub>, R'<sub>1</sub> and R'<sub>2</sub> can be taken together to represent the atoms necessary to complete at least one heterocyclic ring.

33. The developer of claim 31 wherein the benzimidazole is of the structure:



wherein R<sub>4</sub> is hydrogen, nitro or alkoxy and R<sub>11</sub> is hydrogen or lower alkyl.

34. The developer of claim 33 wherein the benzimidazole is spiro [benzimidazoline-2,1'-cyclohexane].

35. The developer of claim 33 wherein the benzimidazole is spiro [5nitrobenzimidazoline-2,1'-cyclohexane].

36. The developer of claim 33 wherein the benzimidazole is spiro [5-methoxybenzimidazoline-2,1'-cyclohexane].

37. The developer of claim 33 wherein the benzimidazole is spiro [benzimidazoline-2,1'-(4'-methylcyclohexane)].

38. The developer of claim 31 wherein the benzimidazole is of the structure:



wherein R<sub>1</sub> and R<sub>2</sub> are substituted acetyl and R<sub>4</sub> and R<sub>5</sub> are independently selected from the group consisting of hydrogen, alkyl and alkoxy.

39. The developer of claim 38 wherein the benzimidazole is 1,3-bistrifluoroacetyl-2,3-dihydrobenzimidazole.

40. The developer of claim 38 wherein the benzimidazole is 5-methoxy-1,3-bistrifluoroacetyl-2,3-dihydrobenzimidazole.

41. The developer of claim 38 wherein the benzimidazole is 5,6-dimethyl-1,3-bistrifluoroacetyl-2,3-dihydrobenzimidazole.

\* \* \* \* \*